

May 7, 1946.

E. J. HOUDRY ET AL

2,399,678

CATALYSIS

Filed July 27, 1943



INVENTOR  
EUGENE J. HOUDRY  
HUBERT A. SHABAKER  
BY *Ira L. Nickerson*  
ATTORNEY

## UNITED STATES PATENT OFFICE

2,399,678

## CATALYSIS

Eugene J. Houdry, Ardmore, and Hubert A. Shabaker, Media, Pa., assignors to Houdry Process Corporation, Wilmington, Del., a corporation of Delaware

Application July 27, 1943, Serial No. 496,286

4 Claims. (Cl. 260—680)

The present invention relates to improvements in catalytic dehydrogenation of hydrocarbons, such as paraffinic, olefinic or alkyl aromatic hydrocarbons which contain a carbon chain of less than 6 carbon atoms.

Catalytic dehydrogenation of the type to which the present invention relates proceeds with the formation of coke or coke-like material which is deposited in the catalyst and the formation of hydrogen in addition to the production of unsaturated or aromatic products. This coke-like material is, of course, formed from the hydrocarbon being dehydrogenated and therefore represents a loss of material. Any reduction in losses, in general, is an advantage. Reduction of coke is of particular advantage in these dehydrogenation processes in facilitating temperature control, and, in the case of adiabatic operation, in improving the conditions of operation.

In modern gas dehydrogenation procedures the heat produced by burning of this coke-like material during regeneration is stored in the catalyst mass and is employed to maintain the temperature during the endothermic dehydrogenation, processes of this type being termed adiabatic dehydrogenations. In these processes a limiting factor on the extent of the dehydrogenation, and therefore the efficiency of the process is the amount of coke produced in relation to the amount of dehydrogenation effected. Thus, as the temperature of the operation increases, the extent of the dehydrogenation in general also increases; likewise, the amount of coke deposited increases. As the temperature is increased, the increase in the amount of coke deposited is more than proportionate to the increase in dehydrogenation. Therefore, under fixed operating conditions, the condition at which the heat of dehydrogenation is equal to the heat of regeneration is a special case. If the ratio of coke deposited to dehydrogenation effected can be decreased, the temperature is increased at which the heat of dehydrogenation is equal to the heat of regeneration. This, accordingly, allows operation of adiabatic operation at higher temperatures, with resultant increase in the extent of dehydrogenation. Likewise, plants operating at high temperatures and using extraneous means to dissipate heat such as an air blow can be run at a substantial saving by a reduction in the ratio of coke to dehydrogenation.

The present invention is of particular application to dehydrogenation processes for the production of butadiene. Dehydrogenation catalysts treated in accordance with this invention not only produce less coke but, additionally, when employed under the same conditions, produce a higher conversion to butadiene, as reflected by higher concentration. Increased concentration is of real and substantial importance since even

a slight increase results in major savings in the cost of recovery of butadiene from mixed dehydrogenation product.

Objects of the present invention are to provide improved processes for the manufacture of dehydrogenation catalysts, to provide improved dehydrogenation processes wherein the losses are decreased, to provide for the use of more favorable operating conditions, and to provide processes for the production of dienes, in particular butadiene, in which, under like conditions, the concentration of diene in the reaction mixture is increased. Other and more specific objects will become apparent as the following description proceeds.

The improvements here involved are applicable in the dehydrogenation of paraffinic hydrocarbons. The product may be principally olefins, as in the dehydrogenation of propane or isobutane to propylene or isobutene, or the product, alternatively, may contain dienes, as in the dehydrogenation of paraffins and olefins to olefins and dienes. Further, the product may contain unsaturated aromatic derivatives, as in the dehydrogenation of alkyl aliphatics in which the alkyl group is a carbon chain containing less than six carbon atoms in the chain. In the latter type of process, the charge may be relatively pure, such as a technical ethylbenzene or it may be a naphtha cut.

This invention involves the treatment of dehydrogenation catalysts of the type which contains a polyvalent, multivalent heavy metal oxide, for example, chromium, molybdenum, vanadium or iron, carried by surface active support comprising a refractory metal oxide, non-reducible under the reaction conditions employed for the dehydrogenation, such as alumina, zirconia, magnesium oxide, and cerium oxide. This treatment of the dehydrogenation catalysts of the type stated is effected at elevated temperature in the presence of steam. The treatment is effected at a temperature between 1200° and 1600° F. at a partial pressure of steam in pounds per square inch above 1 lb. and above

$$\frac{400}{T-1160} - 1$$

and at a partial pressure of steam in pounds per square inch below 30 lbs. and below

$$\frac{475}{T-1630} + 32$$

where T equals the temperature of treatment in degrees Fahrenheit. The treatment is continued for over two hours and for a time sufficient that the ratio of percent dehydrogenation to per cent coke is increased at least 50%, per cent dehydrogenated being calculated as the per cent of dehydrogenated product times one hundred divided by the total of dehydrogenated product plus un-

converted charge. It is in general unnecessary to treat for over thirty hours to obtain the desired change in catalyst characteristics and accordingly it is preferred that the treatment be not extended beyond that time.

It appears that in the preliminary stages of treatment the selectivity of the catalyst is somewhat improved with respect to side reactions which give gas and low boiling hydrocarbons of a number of carbon atoms to the molecule other than contained in the charge. However, upon continued treating, and in accord with this invention, the coke is also reduced. Both of these changes reduce losses. The second one appears to be a permanent change in the catalyst, the results of which are in no way similar to the deposition of a transitory molecular film of water. As an incident of the reduction in coke as stated it has been found that there is an increase in the extent of dehydrogenation.

It should be noted in connection with the mathematical expressions employed to define the treating conditions that these expressions are purely empirical and define the curved lines BC and EF, respectively in the accompanying drawing. Thus, along the line BC the partial pressure of steam is equal to

$$\frac{400}{T-1160} - 1$$

and along the line EF the partial pressure is equal to

$$\frac{475}{T-1630} + 32$$

In this drawing the zone of treating is outlined in heavy lines and consists of the zone ABCDEF.

This invention is illustrated in the following examples which should be taken as indicative of the character of the invention but not definitive of the scope thereof.

#### EXAMPLE 1

Six parts by weight of surface active alumina such as is sold on the market as "Activated Alumina" was soaked for 30 minutes in 8.61 parts by weight of a chromic acid solution of 1.428 specific gravity. The excess solution was then drained off and the pellets were dried in circulating air at 210° F. By analysis the pellets contained 18.5% by weight Cr<sub>2</sub>O<sub>3</sub> on ignited basis. The pellets were divided into three lots. One of the lots employed as a blank was heat treated at 1400° F. for 10 hours in dry air, the other two lots were steam treated in accordance with this invention, one at 1400° for 10 hours at a steam pressure of 3 lbs. and the other at 1400° F. for 20 hours at a steam pressure of 1.5 lbs. The 3 lb. and 1.5 lb. steam pressures were obtained by maintaining the pellets in contact respectively with a 20% steam, 80% air mixture and a 10% steam, 90% air mixture, both of which were maintained at atmospheric pressure. The heat treated catalysts were subjected to reduction by contacting at elevated temperature with hydrogen prior to use for dehydrogenation.

The conditions employed for dehydrogenation were as follows: A mixture of 24.5% n-butane, 75.0% n-butene and 0.5% butadiene was contacted with the catalyst at a temperature of 1075° F., at a pressure of 5 inches mercury absolute and a rate of about 20 grams of charge per liter of catalyst per minute. Each run on a catalyst was conducted for 10 minutes and the catalysts were reduced with hydrogen before each run following regeneration.

The results of dehydrogenation in contact with the three lots of catalysts so prepared are shown in the following tabulation:

Table 1

|    |                                           |       |                   |
|----|-------------------------------------------|-------|-------------------|
| 5  | Temp., °F.....                            | 1,400 | 1,40 <sup>0</sup> |
|    | Time in hours.....                        | 10    | 20                |
|    | Steam pressure.....                       | 3     | 1.5               |
|    | C <sub>4</sub> , C <sub>5</sub> .....     | 6.2   | 0.7               |
|    | Total C <sub>4</sub> .....                | 87.8  | 94.1              |
|    | Butadiene.....                            | 14.8  | 21.0              |
| 10 | Coke.....                                 | 3.4   | 2.0               |
|    | Percent dehydrogenated <sup>1</sup> ..... | 16.8  | 22.3              |
|    | Percent dehydrogenated/coke.....          | 4.94  | 11.1              |
|    | Percent increase in ratio.....            | 125   | 105               |

<sup>1</sup> Percent dehydrogenated =  $\frac{\text{butadiene}}{\text{total C}_4} \times 100$ .

15 It is to be noted that while the catalyst treated for 20 hours at 1.5 pounds steam partial pressure was satisfactory, it was impossible to obtain satisfactory results by treatment under the same conditions for only two hours. After two hours 20 the activity of the catalyst was improved as indicated by the production of 22.9% butadiene, but it produced 3.5% coke, substantially the same as if it had not been heat treated. In this instance the per cent increase in the ratio is 31%.

25

#### EXAMPLE 2

Six parts by volume of "Activated Alumina" pellets were allowed to stand in four parts by volume of a solution of chromic acid of specific 30 gravity 1.025. After standing for 30 minutes the solution was drained from the pellets. There was recovered 1.995 parts by volume of solution of specific gravity 1.018. The pellets were dried at 200° to 210° F. in circulating air and were 35 found to contain 3.28% Cr<sub>2</sub>O<sub>3</sub> on ignited basis.

The dried alumina pellets containing chromic acid were divided into 3 portions, one of which for control purposes was heat treated in dry air for 10 hours at 1400° F. The remaining two portions 40 were steam treated at 1400° F. for 10 hours, one of them at a partial pressure of steam of 1.5 and the other of 3 lbs. per square inch. This steam treat was effected in the first instance by maintaining an atmosphere of 10% steam, 90% air at atmospheric pressure in contact with the catalyst, and in the second instance, 20% steam, 80% air, at atmospheric pressure. After reduction the three catalysts were employed for dehydrogenation under the conditions stated in 45 Example 1. The results tabulated below were 50 obtained:

Table 2

|    |                                       |       |       |
|----|---------------------------------------|-------|-------|
| 55 | Temp., °F.....                        | 1,400 | 1,400 |
|    | Time in hours.....                    | 10    | 10    |
|    | Steam pressure.....                   | 1.5   | 3     |
|    | C <sub>4</sub> , C <sub>5</sub> ..... | 8.6   | 2.6   |
|    | Total C <sub>4</sub> .....            | 84.9  | 90.9  |
|    | Butadiene.....                        | 11.4  | 13.9  |
|    | Coke.....                             | 3.3   | 2.9   |
|    | Percent dehydrogenated.....           | 9.68  | 15.3  |
|    | Percent dehydrogenated/coke.....      | 2.93  | 5.27  |
|    | Percent increase in ratio.....        | 80    | 420   |

#### EXAMPLE 3

Six parts by volume of "Activated Alumina" pellets were soaked for 30 minutes in four parts by volume of a 1.268 specific gravity chromic acid 65 solution, following which residual solution was drained from the pellets. There were 2.15 liters of residual solution of specific gravity 1.285. The pellets were dried in circulating air at 200 to 210° F. The pellets were found by analysis to contain 70 13.68% Cr<sub>2</sub>O<sub>3</sub> on ignited basis.

The dried pellets were divided into four lots and heat treated under the following conditions: The first at 1400° F. for 10 hours in dry air for a blank, the second at 1400° for 10 hours at a steam pressure of 1.5, the third at 1400° F. for 10 hours

at 3 lbs. steam pressure, and the fourth at 1400° F. for 10 hours at 15 lbs. steam pressure. After reduction the catalyst was employed for dehydrogenation under the conditions in Example 1. The results are shown in the following tabulation:

Table 3

| Temp., ° F.                       | 1,400 | 1,400 | 1,400 |
|-----------------------------------|-------|-------|-------|
| Time in hours                     | 10    | 10    | 10    |
| Steam pressure                    | 1.5   | 3     | 15    |
| C <sub>8</sub> , C <sub>9</sub> + | 1.5   | 0.9   | 2.1   |
| Total C <sub>4</sub>              | 90.9  | 94.4  | 93.0  |
| Butadiene                         | 13.8  | 21.9  | 19.7  |
| Coke                              | 4.7   | 3.2   | 3.0   |
| Percent dehydrogenated            | 15.32 | 23.2  | 21.2  |
| Percent dehydrogenated/coke       | 3.27  | 7.25  | 7.07  |
| Percent increase in ratio         | 122   | 116   | 214   |

## EXAMPLE 4

32 liters of "Activated Alumina" pellets were soaked for 30 minutes in 28.6 kilograms of a chromic acid solution of specific gravity 1.142. The remaining solution was then drained off and upon measurement there was obtained 13.05 liters of residual solution of specific gravity 1.146. The pellets were dried at 210° F. in circulating air. The pellets were found by analysis to contain 9.12% Cr<sub>2</sub>O<sub>3</sub> on ignited basis.

The catalyst was divided into four lots and heat treated as stated in Example 3 and employed for dehydrogenation under the conditions in Example 1. The results are shown in the following tabulation:

Table 4

| Temp., ° F.                       | 1,400 | 1,400 | 1,400 |
|-----------------------------------|-------|-------|-------|
| Time in hours                     | 10    | 10    | 10    |
| Steam pressure                    | 1.5   | 3     | 15    |
| C <sub>8</sub> , C <sub>9</sub> + | 3.5   | 2.7   | 0.8   |
| Total C <sub>4</sub>              | 90.6  | 92.3  | 94.8  |
| Butadiene                         | 16.3  | 19.7  | 19.9  |
| Coke                              | 3.4   | 2.5   | 2.4   |
| Percent dehydrogenated            | 18.0  | 21.4  | 21    |
| Percent dehydrogenated/coke       | 5.30  | 8.57  | 8.75  |
| Percent increase in ratio         | 62    | 65    | 72    |

Preferred catalysts employed in the present invention contain a minor portion generally in the range between 2% and 40% of the heavy metal oxide and a major proportion generally in the range from 60% to 98% of the refractory surface active support.

We claim as our invention:

1. The process of dehydrogenating a selected hydrocarbon containing an aliphatic chain of less than 6 carbon atoms which comprises subjecting said hydrocarbon to contact with a dehydrogenation catalyst of the type which contains a polyvalent, multivalent heavy metal oxide carried by a surface active refractory metal oxide support, said catalyst having been preconditioned by contact with steam at a temperature between 1200° and 1600° F. at a partial pressure of steam in pounds per square inch between 1 pound and 30 pounds and above

$$\frac{400}{T-1160}-1$$

and below

$$\frac{475}{T-1630}+32$$

where T equals the temperature of preconditioning in degrees Fahrenheit, the preconditioning being continued for more than two hours and for a time sufficient that the ratio of percent dehydrogenation to percent coke is increased at least 50% over the results obtained with no preconditioning.

2. The process of dehydrogenating a selected hydrocarbon gas which comprises subjecting said gas to contact with a dehydrogenation catalyst of the type which contains a polyvalent, multivalent heavy metal oxide carried by a surface active refractory metal oxide support, said catalyst having been preconditioned by contact with steam at a temperature between 1200° and 1600° F. at a partial pressure of steam in pounds per square inch between 1 pound and 30 pounds, the partial pressure of steam being correlated with the temperature to lie within the zone ABCDEF in the accompanying drawing, the preconditioning being continued for more than two hours and for a time sufficient that the ratio of percent dehydrogenation to percent coke is increased at least 50% over the results obtained with no preconditioning.

3. The process of dehydrogenating a selected hydrocarbon gas which comprises subjecting said gas to contact with a dehydrogenation catalyst which contains a minor portion of chromium oxide carried by a major portion of a surface active alumina, said catalyst having been preconditioned by contact with steam at a temperature between 1200° and 1600° F. at a partial pressure of steam in pounds per square inch between 1 pound and 30 pounds, and above

$$30 \quad \frac{400}{T-1160}-1$$

and below

$$\frac{475}{T-1630}+32$$

where T equals the temperature of the preconditioning in degrees Fahrenheit, the preconditioning being continued for more than two hours and for a time sufficient that the ratio of percent dehydrogenation to percent coke is increased at least 50% over the results obtained with no preconditioning.

4. The process of dehydrogenating a selected hydrocarbon gas which comprises subjecting said gas to contact with a dehydrogenation catalyst of the type which contains a polyvalent, multivalent heavy metal oxide carried by a surface active refractory metal oxide support, said catalyst having been preconditioned by contact with steam at a temperature between 1200° and 1600° F. at a partial pressure of steam in pounds per square inch between 1 pound and 30 pounds, and above

$$55 \quad \frac{400}{T-1160}-1$$

and below

$$\frac{475}{T-1630}+32$$

where T equals the temperature of the preconditioning in degrees Fahrenheit, the preconditioning being continued for more than two hours and for a time sufficient that the ratio of percent dehydrogenation to percent coke is increased at least 50% over the results obtained with no preconditioning.

EUGENE J. HOUDRY.  
HUBERT A. SHABAKER.